

## UNITED STATES PATENT OFFICE

2,453,881

## INHIBITION OF CORROSION IN WELLS

Prentiss S. Viles and Elza Q. Camp, Goose Creek, Tex., assignors to Standard Oil Development Company, a corporation of Delaware

No Drawing. Application January 24, 1946,  
Serial No. 643,206

4 Claims. (Cl. 252—8.55)

1

The present invention is directed to the production of fluids from underground formations. More particularly, the invention is directed to protecting the conduits and attendant equipment, through which fluids from subsurface formations are flowed and processed, from corrosion by materials occurring in or are introduced into fluids originating in subsurface formations.

In many oil, gas, and condensate fields, the production of fluids from subsurface formations is accompanied by extremely severe corrosion of the conduits and attendant equipment which comes into contact with the fluid mixture being produced. In many cases it is found that the fluid mixture is acidic in nature and comprises substantial amounts of carbon dioxide, a portion of which dissolves in water present to form carbonic acid. In addition to the carbon dioxide other materials which are present in the corrosive mixture may include organic acids, inorganic acids, inorganic salts and acidic sulfur compounds. These corrosive substances occur in or are introduced into the fluids originating in the subsurface formations. In some cases the corrosion occurs throughout the conduits and attendant equipment through which the fluids from the subsurface formations are flowed and processed. In other cases the corrosion is limited primarily to portions of the conduits near the surface of the wells and to the wellhead and attendant equipment. In all cases it has been necessary to make extensive replacements of equipment that has failed as a result of corrosion. This not only limits production, but is extremely expensive, particularly in those cases in which it is necessary to kill a high pressure well in order to make repairs and to replace corroded equipment. In addition to the high costs of making repairs to well equipment, there is a marked loss in revenues due to having a well off production and to the necessity of having to maintain additional wells and sources of supply to meet production requirements during periods in which a well is off production for repairs as a result of corrosion. Further, there is constant danger that a well will flow wild as a result of the failure of equipment due to corrosion. In cases of this kind, enormous losses are incurred.

It is, therefore, the main object of the present invention to provide a method whereby corrosion is substantially eliminated or inhibited in the conduits and attendant equipment through which fluids from subsurface formations are flowed and processed.

In accordance with the present invention, cor-

2

rosion of ferrous metal surfaces is inhibited or substantially eliminated by adding to fluid mixtures produced from subsurface formations and which are acidic in nature and include carbon dioxide a small amount of carbon disulfide. The amount of carbon disulfide employed to inhibit the corrosion of the ferrous metallic surfaces by the fluid mixtures may be varied over a wide range and satisfactory results obtained. Inasmuch as sulfur-containing compounds are usually undesirable constituents in the hydrocarbon fluid being obtained, it is preferable to employ only small amounts of carbon disulfide to inhibit the corrosion but in some cases relatively large amounts of the carbon disulfide may be desirable or necessary and in such instances it may be added in amounts up to 3% by weight based on the weight of fluid mixture produced from the subsurface formation. However, it will usually be found that minor amounts of carbon disulfide will be effective for inhibiting corrosion of the ferrous metal surfaces and, accordingly, under many operation conditions carbon disulfide used for effectively inhibiting corrosion may be .1% or even as low as .01% by weight of the fluid mixture being produced.

It may be found that after an effective amount of carbon disulfide has been employed to inhibit corrosion of the ferrous metal surface, a lower amount may be effective thereafter to maintain the inhibiting effect. Accordingly, a substantial amount of carbon disulfide, as of the order of 1% by weight of the fluid produced, may be employed for an interval of time sufficient to cause corrosion of the metallic surfaces to be effectively inhibited and thereafter smaller amounts, as of the order of .01% of carbon disulfide based on the weight of the fluid produced, may be employed to maintain the inhibited condition of the metallic surfaces.

It will be found convenient to suspend or dissolve the carbon disulfide in a suitable vehicle before introducing it into the fluid mixture. The resultant suspension or solution may then be conveniently injected into the borehole adjacent the subsurface formation from which the fluid is produced or may be introduced into the conduit through which the fluid mixture flows from a subsurface formation to the surface of the earth. Another method of employing the inhibiting agent is by injecting the suspension or solution into the subsurface reservoir by employing an adjacent well; it will be apparent that when adding the inhibiting agent in accordance with this procedure the fluid entering the bore-

hole of the producing well will comprise the inhibiting agent.

An advantage of the process of the present invention, irrespective of the suppression of corrosion of the conduits and attendant equipment through which fluids from subsurface formations are flowed and processed, is the ability to operate without interruptions due to failure of equipment. The danger of a well flowing wild is minimized and the necessity of having a surplus of wells to insure production is eliminated.

In order to illustrate further the beneficial effects of the present invention, the following examples are given:

**EXAMPLE I**

Test pieces of carbon steel were immersed in water solutions under a pressure of 100 lbs. per sq. in. gauge of carbon dioxide and the test pieces were maintained under this pressure for an interval of 24 hrs. and at a temperature of 170° F. The carbon dioxide was admitted to the system through a pressure regulator valve thus maintaining a constant pressure of carbon dioxide on the system so that the water solutions in which the carbon steel test specimens were immersed were saturated with carbon dioxide at the temperatures and pressures at which the tests were conducted. One of the solutions was employed as a blank with no inhibiting material added while the other solution had carbon disulfide added thereto. The results obtained by the test are shown in Table I.

**Table I**

| Inhibiting Material   | Amount of Inhibiting Material, Per Cent by Wt. | Corrosion Rate, In. per Yr. | Reduction of Corrosion by Inhibition, Per Cent |
|-----------------------|------------------------------------------------|-----------------------------|------------------------------------------------|
| None.....             | None                                           | 0.2250                      | .....                                          |
| Carbon Disulfide..... | 1.0                                            | 0.0269                      | 88.1                                           |

In order to determine the effectiveness of alternating the pressure on the inhibiting agent, a series of tests was conducted as follows:

**EXAMPLE II**

A quantity of distilled water was divided into a plurality of samples. Some of the samples were maintained as distilled water; to other of the samples acetic acid was added to obtain a pH of 4.5; to other samples of distilled water hydrochloric acid was added to obtain a pH of 4.5; in other samples a low concentration of sodium chloride was dissolved, while to still other samples a high concentration of sodium chloride was dissolved. Some of the samples were then inhibited by adding CS<sub>2</sub> thereto. Test pieces of carbon steel were immersed in the solutions prepared. One set of samples was then maintained under the pressure of 100 lbs. per sq. in. gauge of carbon dioxide, a second set of samples was maintained under a pressure of 500 lbs. per sq. in. gauge of carbon dioxide while a third set of the samples was maintained under a pressure of 900 lbs. per sq. in. gauge of carbon dioxide. In conducting the tests the sets of samples were maintained under superatmospheric pressure for an interval of 24 hours and at a temperature of 170° F. The results obtained when conducting the tests under a pressure of 100 lbs. per sq. in. are set forth in Table II below; the results obtained when conducting the tests under a pressure of 500 lbs. per sq. in. are shown in Table III below, while the results obtained when conduct-

ing the tests under a pressure of 900 lbs. per sq. in. are shown in Table IV below.

**Table II**

| Type of Solution                                               | Corrosion Rate, Inch Per Year |                                                 | Reduction in Corrosion Rate, Percent |
|----------------------------------------------------------------|-------------------------------|-------------------------------------------------|--------------------------------------|
|                                                                | Without Inhibitor             | Inhibited With 1 Wt. Percent of CS <sub>2</sub> |                                      |
| Distilled Water.....                                           | 0.2250                        | 0.0269                                          | 88.0                                 |
| Distilled Water Adjusted to pH 4.5 with Acetic Acid.....       | 0.1869                        | 0.0175                                          | 90.7                                 |
| Distilled Water Adjusted to pH 4.5 with Hydrochloric Acid..... | 0.0555                        | 0.0166                                          | 71.0                                 |
| Water of Low Salt Content.....                                 | 0.1199                        | 0.0209                                          | 82.0                                 |
| Water of High Salt Content.....                                | 0.1098                        | 0.0197                                          | 82.0                                 |

**Table III**

| Type of Solution                                               | Corrosion Rate, Inch Per Year |                                                 | Reduction in Corrosion Rate, Percent |
|----------------------------------------------------------------|-------------------------------|-------------------------------------------------|--------------------------------------|
|                                                                | Without Inhibitor             | Inhibited With 1 Wt. Percent of CS <sub>2</sub> |                                      |
| Distilled Water.....                                           | 0.2083                        | 0.0278                                          | 86.8                                 |
| Distilled Water Adjusted to pH 4.5 with Acetic Acid.....       | 0.1070                        | 0.0164                                          | 86.6                                 |
| Distilled Water Adjusted to pH 4.5 with Hydrochloric Acid..... | 0.0343                        | .....                                           | .....                                |
| Water of Low Salt Content.....                                 | 0.1073                        | 0.0189                                          | 82.0                                 |
| Water of High Salt Content.....                                | 0.0447                        | .....                                           | .....                                |

**Table IV**

| Type of Solution                                               | Corrosion Rate, Inch Per Year |                                                 | Reduction in Corrosion Rate, Percent |
|----------------------------------------------------------------|-------------------------------|-------------------------------------------------|--------------------------------------|
|                                                                | Without Inhibitor             | Inhibited With 1 Wt. Percent of CS <sub>2</sub> |                                      |
| Distilled Water.....                                           | 0.2100                        | 0.0219                                          | 89.5                                 |
| Distilled Water Adjusted to pH 4.5 with Acetic Acid.....       | 0.1060                        | 0.0401                                          | 62.3                                 |
| Distilled Water Adjusted to pH 4.5 with Hydrochloric Acid..... | 0.0310                        | .....                                           | .....                                |
| Water of Low Salt Content.....                                 | 0.1307                        | 0.0179                                          | 86.3                                 |
| Water of High Salt Content.....                                | 0.0182                        | .....                                           | .....                                |

It will be observed from the data presented above that the addition of a small amount of carbon disulfide effects a marked reduction in the tendency of a corrosive water solution to corrode carbon steel. It is to be noted that all sulfur-containing compounds are not effective for inhibiting corrosion of ferrous metallic surfaces when exposed to corrosive fluids produced from subsurface formations. For example, ethyl sulfate is entirely ineffective in inhibiting the corrosion of ferrous metallic surfaces by such fluids.

The nature and objects of the present invention having been fully described and illustrated, what we wish to claim as new and useful and to secure by Letters Patent is:

1. A method for reducing the corrosiveness to corrodible ferrous metal of a corrosive petrolierous well fluid including moisture and carbon dioxide which comprises introducing into said fluid a corrosion inhibiting amount of carbon disulfide.

2. A method in accordance with claim 1 in which the carbon disulfide is added to the corrosive fluid in an amount no greater than 1% by weight.

3. A method in accordance with claim 1 in which the carbon disulfide is introduced into the corrosive fluid in a subsurface formation at a point remote from the point at which the fluid is produced.

4. A method in accordance with claim 1 in which the corrosive fluid is produced from a subsurface formation through a ferrous metal conduit and in which the carbon disulfide is introduced directly into said conduit.

PRENTISS S. VILES.  
ELZA Q. CAMP.

## REFERENCES CITED

The following references are of record in the 15 file of this patent:

## UNITED STATES PATENTS

|   | Number    | Name      | Date          |
|---|-----------|-----------|---------------|
| 5 | 1,829,705 | Walker    | Oct. 27, 1931 |
|   | 1,844,883 | De Groote | Feb. 9, 1932  |
|   | 1,873,084 | Walker    | Aug. 23, 1932 |
|   | 2,357,559 | Smith     | Sept. 5, 1944 |

## OTHER REFERENCES

10 Formaldehyde vs. Sulfide Corrosion, article in Industrial and Engineering Chemistry, Industrial edition, vol. 38, pages 10 and 14.